

Patented Jan. 10, 1939

2,143,802

# UNITED STATES PATENT OFFICE

2,143,802

## FOG INHIBITORS FOR PHOTOGRAPHIC EMULSIONS

Samuel E. Sheppard and Waldemar Vanselow,  
Rochester, N. Y., assignors to Eastman Kodak  
Company, Rochester, N. Y., a corporation of  
New Jersey

No Drawing. Application January 8, 1937,  
Serial No. 119,660

2 Claims. (Cl. 95—7)

This invention relates to fog inhibitors for photographic emulsions and to photographic emulsions containing them.

It is known that photographic emulsions particularly ultra-sensitive emulsions, or those containing color sensitizers exhibit a tendency to form a deposit of silver in the emulsion. This deposit extends more or less uniformly over the entire emulsion and is known as fog. Photographic fog is of two types, local and general. Local fog is formed by exposure of the film or plate at undesired points, as by a light leak in the camera. General fog or, as it is sometimes known, chemical fog, is formed in a number of ways. It may be caused by the conditions under which the film or plate is stored, such as conditions of high temperature or unusually long time of storage. The nature of the emulsion, as where emulsions are highly sensitive may also produce chemical fog, as well as the conditions of development of the emulsion, as by development for protracted periods of time or at temperatures above normal. Highly sensitive emulsions are more likely to fog than those of lower sensitivity, owing to the small amount of energy required to make a silver halide grain developable. We are concerned primarily with general or chemical fog.

The principal object of the present invention is to provide fog inhibiting agents for photographic emulsions which decrease the tendency of the emulsions to form general or chemical fog and, therefore, increase its stability. A further object is to provide fog inhibiting agents which do not markedly lower the sensitivity of the emulsion.

These objects are accomplished by incorporating in the emulsion suitable amounts of a morpholine compound, such as phenyl morpholine.

We have found that not all morpholine compounds are useful for preventing the fogging of photographic emulsions, but only certain of the morpholine compounds serve to inhibit the fogging tendency without lowering the sensitivity of the emulsion. For example, while phenyl morpholine has definite fog inhibiting value, compounds such as ethoxy ethyl morpholine have no definite value for this purpose when used under the same conditions as phenyl morpholine.

A compound which we have found useful has the following structural formula:



Phenyl morpholine was found to give very good stabilization at a concentration of about 0.02 gram per 1000 cc. of emulsion and also at concentrations as high as 4 grams per 1000 cc. of emulsion. Variation in the quantity necessary depends upon the type of emulsion, its hydrogen ion concentration, the amount of halide present, and on other factors.

It is to be understood that more or less of the anti-foggant agent and the amounts stated above may be used. Generally, however, if a greater amount is used in the emulsion, either no increased fog inhibiting effect is obtained or there is a loss in sensitivity of the emulsion. The fog inhibiting agents are incorporated by mixing them with any suitable solvent which is inert with respect to the sensitive emulsion, such as ethyl alcohol or other liquid in which the compound was soluble. An ethyl alcohol solution of 1% strength of phenyl morpholine was found to be suitable for incorporation of the compounds which we propose to use.

The following example which is by way of illustration only indicates methods of incorporating the fog inhibiting agents in photographic emulsions according to our invention.

### Example I

A gelatino-silver halide negative emulsion which had been made in the usual way was heated on a water bath to a sufficient temperature to melt it. To a 1000 cc. portion of this emulsion there was added a solution of 100 cc. of ethyl alcohol containing 1 gram of phenyl morpholine. The resulting solution was thoroughly mixed and was coated on glass plates, dried and incubated for about a week at 60° C. to obtain a fog test. There was found to be a marked fog inhibiting result through the use of the phenyl morpholine, as compared with a similar emulsion to which no fog inhibiting agent had been added.

The fog inhibiting agents which we have described may be used in various kinds of photographic emulsions. In addition to being useful in ordinary non-color sensitized emulsions they may also be used in orthochromatic, panchromatic and X-ray emulsions. They may be used with or without color sensitizing dyes and if used with the sensitizing dyes they may be added to the emulsion before or after the dyes are added. Various silver salts may be used as the sensitive salt, such as silver bromide, silver iodide, silver chloride or mixtures of these. The dispersing agent may be gelatin or other colloids, such as

collodion, albumin, or suitable cellulose organic derivatives or artificial resins.

It is to be understood that we contemplate as included within our invention all modifications and equivalents coming within the scope of the appended claims.

What we claim and desire to secure by Letters Patent of the United States is:

1. A photographic silver halide emulsion containing phenyl morpholine as an anti-foggant.
2. A gelatino-silver halide emulsion containing as an anti-foggant, about 0.04 gram to about 4 grams per 1000 cc. of emulsion of phenyl morpholine.

**SAMUEL E. SHEPPARD.**  
**WALDEMAR VANSELOW.**